# EUROPEAN PATENT SPECIFICATION

(11) **EP 1 543 172 B1**
(45) Date of publication and mention of the grant of the patent: **16.12.2009**
(21) Application number: 03753690.1
(22) Date of filing: 24.09.2003
(51) Int. Cl.: C22B 34/12, C22B 9/22, C22B 9/14, C25C 3/28, B22F 5/00, B22F 3/18

(54) **PURIFICATION OF METAL PARTICLES BY HEAT PROCESSING**
REINIGUNG VON METALLPARTIKELN DURCH HITZEBEHANDLUNG
PURIFICATION DE PARTICULES MÉTALLIQUES PAR TRAITEMENT THERMIQUE

(30) Priority: 25.09.2002 GB 0222219; 26.09.2002 GB 0222358; 26.09.2002 GB 0222348
(43) Date of publication of application: 22.06.2005
(73) Proprietor: Metalysis Limited, Manvers Way Wath Upon Dearne Rotherham S63 5DB (GB)
(72) Inventor: WARD-CLOSE, Charles Malcolm QinetiQ Limited, Farnborough GU14 0LX (GB); GODFREY, Alastair Bryan QinetiQ Limited, Farnborough GU14 0LX (GB); GOODWIN, Paul Stephen Casting Technology Int., Sheffield S2 3PT (GB)
(74) Representative: Goodman, Simon John Nye
(86) International application number: PCT/GB2003/004093
(87) International publication number: WO 2004/029332

(56) References cited:
- EP-A- 0 047 665
- EP-A- 0 153 296
- GB-A- 2 359 564
- US-A- 3 442 321
- US-A- 4 114 251
- US-A- 4 612 179
- US-A- 4 727 928
- US-A- 5 147 451
- MAC RAE D R: "PLASMA ARC PROCESS SYSTEM, REACTORS, AND APPLICATIONS" PLASMA CHEMISTRY AND PLASMA PROCESSING, PLENUM PRESS. NEW YORK, US, vol. 9, no. 1, SUPPL, 1 March 1989 (1989-03-01), pages 85S-118, XP000117580 ISSN: 0272-4324
- BOMBERGER H B: "The melting of titanium" JOURNAL OF METALS - JOM, METALLURGICAL SOCIETY OF THE AIME. NEW YORK, US, vol. 36, no. 12, 1 December 1984 (1984-12-01), pages 39-47, XP002086633
- PATENT ABSTRACTS OF JAPAN vol. 0124, no. 62 (C-549), 5 December 1988 (1988-12-05) & JP 63 183145 A (SUMITOMO ELECTRIC IND LTD), 28 July 1988 (1988-07-28)

## Description

This invention relates to a method for the purification of metal particles, for example, metal powders and other finely sized metal samples, and, in particular, to ones that have been produced by the process of electrochemical reduction of metal compounds. The invention is particularly suited to the purification of titanium powder formed from the electrolytic reduction of titanium oxide TiO₂.

WO 99/64638 describes methods for the electrolytic reduction (or "electro-reduction") of metal compounds. Certain embodiments of those methods involve the electrolysis of metal oxides or other compounds in a cell containing a liquid (fused salt) electrolyte and an anode, the metal oxide forming or contacting the cathode. Conditions are controlled so as to bring about the selective dissolution of the oxygen of the cathode in preference to deposition of the metal cation of the fused electrolyte. The metals extracted by such methods, however, often require further purification.

GB2359564 is directed to improved methods for carrying out such processes, particularly to produce powdered titanium, and some of those methods are summarised below:-

### Production of powder by reduction of sintered metal oxide granules

Sintered granules or powders of metal oxide can be used as the feedstock for the electrolysis described in the above referenced method, as long as appropriate conditions are present. In one example, powdered titanium dioxide in the form of granules or a powder is used, the powdered particles preferably having a size in the region of 200µm.

As illustrated in Figure 1, the granules of titanium dioxide 1 are held in a basket 2 below a carbon anode 3 located in a crucible 4 having a molten salt 5 therein. These are prevented from sintering together by maintaining particle motion by any appropriate method e.g. in a fluidised bed arrangement. Agitation is provided either by mechanical vibration or by the injection of gas underneath the basket. Mechanical vibration can, for example, be provided by ultrasonic transducers mounted on the outside of the crucible or on control rods. The key variables to be adjusted are the frequency and amplitude of the vibrations in order to get an average particle contact time which is long enough to get reduction, but short enough to prevent diffusion bonding of the particles into a solid mass. Similar principles would apply to agitation by the injection of gas, except here the flow rate of the gas and size of the gas bubbles would be the variables controlling particle contact time.

### Production of powder by deposition of M₁ onto the cathode

If a metal is deposited onto a cathode (based on the electrolytic process previously described) from a second source of the metal at a more positive potential, the resulting metal deposited thereon is dendritic in structure. This is particularly so where the metal is titanium. This form of titanium is easy to break up in to a powder as individual particles are connected together only by a small surface area. This method can be used to produce titanium powder from titania. In this method, illustrated in Figure 2, a second cathode 6 is provided which is maintained at a potential that is more negative than the first cathode 7. When the deposition of titanium on the first cathode has progressed sufficiently, the second electrode is switched on, leading to the dissolution of titanium from the first cathode and deposition 8 onto the second cathode 6 in dendritic form. The other reference numerals represent the same items as in Figure 1.

### Use of continuous powder feed

Continuously feeding a fine powder of metal oxide into the electrochemical cell allows for a constant current and a higher reaction rate. A carbon electrode is preferred for this method. This method permits the use of cheaper feedstock as a sintering and/or forming stage is no longer needed.

This method is shown in Figure 3 which shows a conducting crucible 1 which is made the cathode containing a molten salt 2 and inserted therein is an anode 3. Titanium dioxide powder 4 is fed into the crucible where it undergoes reduction and is deposited at the base of the crucible. The thick arrow shows the increasing thickness of the reduced feedstock 5.

In electro-reduction methods such as those exemplified above, the purity of the metal powder may be affected by the starting materials and processing parameters used. For example, it has been found that some variations of the method when used to produce titanium powder result in powder that contains "contaminating impurities" resulting wherefrom, including light metals such as magnesium or calcium, as well as salts such as calcium chloride (the latter being a preferred electrolyte). Such impurities are known to affect the mechanical properties of alloyed metal components, for example, salt inclusions are known to affect the fatigue performance and weldability of titanium alloys.

A consequence of the presence of those contaminating impurities in electrolytically reduced metal powders is that they are unsuitable for use in lower temperature powder metallurgy processes such as sintering or forging which are performed at temperatures below the alloy melting temperature.

Conventional methods for removing contaminants from metals are described in published patent application EP 0047665 and patent number US 4,727,928. In EP 0047665, a charge comprising metal sponge and a sponge-forming reaction product is heated in a retort means to a temperature sufficient to cause evaporation of the reaction products from the metal sponge. The reaction products are then conducted to a condenser means where they are condensed. In US 4,727,928, tantalum or niobium containing volatile impurities, such as sodiothermic tantalum powder or scrap tantalum from capacitor (condenser) anodes, is converted into crude cast metal by plasma melting. The crude cast metal is then submitted to electron beam melting to produce refined cast metal.

### Summary of Invention

The invention provides a method as defined in the appended independent claims, to which reference should now be made. Preferred or advantageous features of the invention are set out in dependent claims.

In accordance with a first aspect of the present invention there is provided a method for purifying metal M₁ particles manufactured by an electrochemical reduction process, the method comprising the steps of:
introducing the metal M₁ particles into a heat source, such that the particles are out of contact with any surfaces, at a temperature substantially equal to or higher than the melting point of M₁ so as to cause vaporisation of some or substantially all of the contaminating impurities present;
removing the vaporised impurities from the vicinity of the particles;
and cooling the purified metal M₁ particles for collection in solid form.

The present invention thus provides a method for purifying electrochemically reduced metal particles so as to reduce or remove the aforementioned "contaminating impurities" introduced by the reduction process, so as to enable, for example, direct use of the electrolytically reduced metals in lower temperature powder metallurgy processes.

It has been found that the kinds of impurities introduced by such electro-reduction processes are usually more volatile than the metal M₁ and may be conveniently removed by the present process. Such impurities may comprise light metals, for example, calcium and magnesium, as well as salts from the electrolyte, such as calcium chloride. For effective removal of impurities without significant loss of metal M₁, the impurities should preferably be more volatile than the metal M₁ by at least a factor of ten, or preferably 20, in terms of their respective vapour pressures at the processing temperature. Preferably, the processing temperature and/or heating time should be sufficient to remove substantially all the contaminating impurities, for example, so as to reduce their total level to less than 50 ppm, or less than 10% their initial total concentration. Preferably the process is conducted so that there is little or no evaporation (for example, less than 5%) of the metal M₁.

Another feature of metal powders produced by electrolytic reduction of oxide or oxides is that the powder particles tend to be irregular in shape, contain internal cavities and have a rough outer surface. For certain powder metallurgy processes these features are undesirable, and a fully dense spherical particle morphology is preferred, for example in order to impart good flowability. Hence, although the particles may only be partially melted in order to remove said impurities, in most cases the particles need to be fully melted to achieve dense, spherical particles.

Desirably, the heat source is arranged such that the metal particles may be allowed to free fall through the heat source. Suitable heat sources include but are not strictly limited to a hot plasma torch, a hot gas flame, a tube furnace, an induction coil, electric arcs and lasers.

In one embodiment of the invention, the particles may be blown through a plasma torch into the flame and allowed to free fall into a collecting vessel. The torch is preferably arranged at a sufficient height above the vessel such that any portion of the particles that is melted by the heat source is substantially solidified before collection. This prevents distortion of the shape of the particles.

In another embodiment the established method of levitation melting may be used to hold particles of powder in a surrounding heat source for a period sufficient to vaporise the impurities. In a further embodiment, zero gravity processing may be used. The common purpose of these embodiments is to suspend the particles individually in mid-air, out of contact with any surfaces, so as to enable particles to be heated and melted and resolidified individually, without contact with each other, or a container.

The temperature of the heat source should be at or above the melting point of the metal M₁. For titanium the desired point is about 1680°C and for titanium alloys approximately 1500-1800°C. It is known that an argon or helium arc plasma torch can achieve temperatures sufficient to melt titanium powder particles entrained in the flame. Ideally, the process is conducted in a controlled atmosphere, for example, at low pressure/vacuum and/or in an inert atmosphere. In the case of Ti it is important that the powder particles are kept separate from oxygen or nitrogen while above a temperature of about 500°C. This is achieved in practice either by processing in a vacuum or in an atmosphere of Ar.

The method is applicable to all metals and alloys provided a temperature sufficient to melt the particles and volatise the contaminants can be achieved.

The step of removing the impurities may simply involve allowing them to be swept away by the gas flow from the flame of the heat source. Preferably, the step of removing the impurities involves condensing the vaporised impurities on cold collector plates positioned adjacent the hot gas flame and disposing of the condensed impurities. Additionally, if the contaminants re-condense onto the surfaces of the powder particles M₁, then they can be removed easily with a water or dilute acid wash.

Aside from improving the purity of the metal powder, the inventors have appreciated that by exposing small particles of a metal M₁ to a heat source at around or above the melting point, but below the boiling point of M₁, and allowing them to fall freely through the heat source, the shape of the particles can be altered to a near spherical shape. Spherical particles provide improved bonding in powder metallurgy processes. Thus it is preferred that the temperature of the heat source used in the purification process of the method is substantially equal to or higher than the melting point of M₁ but lower than the boiling point of M₁.

Powdered particles purified in accordance with the method of the invention may be used in the formation of alloy metal articles made by various powder metallurgy methods and will provide improved particle bonding and mechanical properties in the alloyed article.

In another aspect, the invention provides a method for the manufacture of a metal article containing a metal M₁, by purifying metal M₁ particles as set out in the first aspect of the invention above and performing a powder metallurgy process on the particles to form the article.

This method may advantageously comprise the steps of:
electrochemically reducing a source of a compound of the general formula M₁X to remove substantially all of element X and provide powder particles consisting substantially of metal M₁;
introducing the metal powder M₁ into a heat source at a temperature substantially equal to or higher than melting point of M₁ for a period of time sufficient to cause vaporisation of a significant proportion of the one or more impurities;
removing the vaporised impurities;
cooling the purified metal M₁ powder; and
mixing the purified M₁ powder with powder of other alloy components and,
performing a powder metallurgy process on the mixture to form an alloyed article.

Preferably, the temperature of the heat source will be substantially equal to or above the melting point of the metal M₁.

The electrochemical reduction method may comprise any suitable electro-reduction method for the production of metal particles, and includes the methods described herein or as described in WO 99/64638.

The powder metallurgy process used may be any conventional powder metallurgy process including but not limited to powder sintering and/or forging. One example of such a process is hot isostatic pressing.

Purified powders made according to the first aspect of the invention may be used in various other processes for the manufacture of metal articles where powdered starting materials are desirable.

For the purposes of this specification M₁ may be construed to mean a single metal or a combination of different metals formed in a single method. References to particles may be construed to mean a powder or other finely sized metal samples, for example, granules or pellets, that could be purified by the present method. A powder may be construed to comprise small particles up to about 1mm in diameter.

Examples employing the present invention will now be described in more detail, by way of example only, with reference to the accompanying drawings of which:
Figure 1 shows a prior art electrolytic cell in which the metal oxide to be reduced is in the form of granules;
Figure 2 shows a prior art electrolytic cell in which an additional cathode is provided in order to refine the metal to a dendritic form;
Figure 3 shows a prior art electrolytic cell employing a continuous powder feed;
Figure 4 shows a preferred purification apparatus according to the present invention;
Figure 5 shows an alternative purification apparatus according to the present invention;
Figure 6 shows a schematic illustration of an apparatus for the production of titanium metal or alloy sheet; and,
Figure 7 shows a schematic illustration of an apparatus for the production of titanium metal or alloy bar stock.

Figures 1 to 3 show, by way of example, three suitable prior art arrangements for producing metal powders by electrolytic reduction, and are discussed in more detail above.

Figure 4 shows a preferred arrangement for purifying a powder in which the particles are blown through a plasma torch into a flame and allowed to free fall into a collecting means. The reactor 10 comprises a large metal vessel 11, provided with an inert atmosphere 12, which is preferably argon dispensed from jets 9. For titanium, the process should be entirely contained in a metal vessel in an inert gas atmosphere. The metal particles (M₁) enter the vessel from a supply hopper 14 through the plasma torch 13, which is attached and sealed to the top of the vessel 11 so that it points downwards, and provides sufficient heat to melt and vaporise the metal particles and contaminants, respectively, as they pass through the upper section of the vessel 11. The torch 13 is preferably arranged at a sufficient height above the collecting means that any portion of the particles that is melted by the heat source is substantially solidified before collection. This prevents distortion of the shape of the particles. The re-solidified powder is collected and sealed into a metal collection hopper 15 via a funnel cyclone collector 16.

In the alternative embodiment shown in Figure 5, levitation melting is used to hold particles of powder in a surrounding heat source for a period sufficient to vaporise the impurities. The apparatus comprises a supply hopper 14 through which metal particles (M₁) enter via a valve 24 into a large ceramic tube-like chamber 23. The powder is allowed to fall through the ceramic tube under its own weight. Around the mid-section of the chamber 23 is an external concentric electromagnetic induction coil 22, which both heats and levitates the metal powder particles such that they spend sufficient time at a suitable temperature for volatile contamination removal and spheroidisation to take place. The purified powder then falls to the bottom of the chamber 23, cooling sufficiently to solidify, before exiting via valve 25 and being collected and sealed into a metal canister 15. In a further refinement, an inert gas flow is introduced counter to the direction of the metal powder flow via inlet 21 and outlet 20, and this both enhances the cooling of the powder particles at the lower end of the tube, and also helps to carry away volatile species.

An electro-reduction process, also known as an electro-deoxidation (EDO) process, is less expensive and easier to perform than conventional metal extraction methods. Metal particles produced by an EDO process may advantageously be used directly as feedstocks in manufacturing processes that incorporate the present purification process as an integral stage.

An embodiment of the present invention provides a method for the manufacture of a metal alloy article of uniform cross section comprising the steps of:
introducing a continuous source of metal alloy M₁ pellets, manufactured by an electrochemical reduction process, to a processing means;
heating the pellets as they approach the processing means, by free-fall through a heat source, to a temperature substantially equal to or higher than the melting point of M₁ so as to cause vaporisation of some or substantially all of the contaminating impurities present;
removing the vaporised impurities from the vicinity of the pellets;
drawing the metal through the processing means so as to coalesce the pellets to form the desired article; and,
cooling the cast stock.

Such a manufacturing process has, in particular, significant benefits over conventional processes for the production of titanium articles. Conventional methods for the manufacture of titanium and titanium alloy stock involve hot working of large titanium alloy ingots. The high temperatures and pressures required for these processes contribute to the high cost of this stock compared to other metal products such as steel and aluminium alloys. Titanium is conventionally obtained from its ore by the Kroll route, a complex chlorination and magnesium reduction method. The purified metal granules, called sponge, are then melted with the alloying additions and cast into large titanium alloy ingots. The metal is melted at least twice and sometimes more, in order to ensure chemical homogeneity and freedom from defects. The large titanium alloy ingots are then hot forged repeatedly to produce the semi-finished alloy stock shapes, such as bar, plate, sheet and wire, required for the manufacture of articles.

The present invention aims to provide novel methods for the manufacture of titanium or other metal alloy stock, which are less expensive and easier to perform.

For sheet production, the above-mentioned manufacturing process incorporating the purification stage may involve:
introducing the continuous source of pellets of the metal alloy to a pair of cooled feed rollers;
heating and simultaneously purifying the pellets in the above described manner as they approach the nip of the pair of feed rollers;
drawing the metal through the nip of the rollers to form a sheet of metal alloy; and,
cooling the sheet.

The pellets should be heated sufficiently to allow them to coalesce to form a sheet when subjected to the pressure of the nip, and may be heated so that they soften, or, at least partly melt, or even fully melt. The term "pellet" covers particles ranging from powders to granules.

Preferably either or both of the feed rollers are water cooled by passing a coolant through their centres. One suitable coolant is water, other suitable fluids will no doubt occur to the skilled addressee.

Alternatively, for stock production, the above-mentioned manufacturing process incorporating the purification stage may involve:
introducing the continuous source of pellets of the metal alloy to a shaped crucible;
heating and simultaneously purifying the pellets in the above described manner as they approach the exposed surface of the crucible;
drawing the at least partially molten metal from an opposing surface of the crucible through a die, the die having a cross section of near net shape and dimensions to the desired net shape and dimensions of the required stock; and
cooling the cast stock.

The sheet or cast stock may be allowed to cool or may be actively cooled.

The alloy pellets may be obtained by an electro-deoxidation process such as that described in WO 99/64638, or, in the Applicant's co-pending applications GB2359564 or GB2362164. As is described in the above specifications, electrochemical reduction may be used to provide small pellets of alloy having high purity and good grain structure. Thus, heating and purification involving softening or partially melting the pellets is sufficient to bond the pellets and obtain a mass of alloy having good mechanical properties.

The step of heating the pellets is preferably carried out by means of an energy beam. The energy beam may, optionally, be selected from an electron beam, a laser or a plasma torch.

Preferably, the processing temperature and/or heating time should be sufficient to remove substantially all the contaminating impurities, for example, so as to reduce their total level to less than 50 ppm, or less than 10% their initial total concentration. Preferably the process is conducted so that there is little or no evaporation (for example, less than 5%) of the metal. Ideally, the process is conducted in a controlled atmosphere, for example, at low pressure/vacuum and/or in an inert atmosphere. In the case of Ti it is important that the powder particles are kept separate from oxygen or nitrogen while above a temperature of about 500°C. This is achieved in practice either by processing in a vacuum or in an atmosphere of Ar. The use of argon or helium arc torches is particularly preferred.

In either method, the rolled or cast stock may be further processed, for example, by one or more additional intermediate steps such as further working or heat treatments of the stock, prior to final cooling. Products of the methods are comprised of fully dense metal alloy. The homogeneity of the final metal is improved considerably because the pellets are provided via an electrochemical reduction method, as compared to the alternative of using Kroll sponge and powder or particles of the alloy additions. The present methods require considerably less cumbersome and costly apparatus compared to conventional methods where the starting materials are introduced to the casting or rolling apparatus fully molten and are particularly suited to the production of small quantities of stock where mechanical properties and metal homogeneity are of importance.

The present methods are particularly suited to the manufacture of low volume or small size products, which could be prohibitively costly to produce by conventional methods.

Two embodiments illustrating the roller and crucible based processes will now be further described with reference to Figures 6 and 7.

As can be seen from Figure 6, pellets of titanium metal or alloy 31 are delivered through a hopper 32 to a pair of counter-rotating feed rollers 33a, 33b. The rollers are cooled by a water-cooling system (not shown). An energy beam 34 is arranged to concentrate a beam of energy along a line just above the nip of rollers 33a, 33b and causes at least partial melting of the pellets seated on and between the rollers. As the rollers 33a, 33b rotate, the at least partially melted pellets are drawn into the nip and are squeezed together to form a solid mass of the titanium or titanium alloy in the form of a sheet 35. The hot sheet falls to a conveyor 36 and is carried away for further processing and/or cooling.

Figure 7 illustrates a similar arrangement for the production of bar stock having a square cross-section. A source of pellets 41 is delivered through a hopper 42 to a shallow crucible 47. A laser 44 is mounted on a track 48 along which the energy beam sweeps back and forth. The energy beam is aimed at the top surface of the crucible 47 and causes at least partial melting of the pellets 41 delivered thereto. The metal is drawn through a square shaped die 49 communicating with a lower surface of the crucible 47 and bar stock 45 of the titanium or titanium alloy emerges. The bar stock may be cut to length by a cutter (not shown). The bar stock is collected by a conveyor system 46 and removed for cooling and/or further processing.

The parameters for a method carried using either of the described apparatus are more generally described below.

The feedstock in the form of pellets (including powder or granules) is stored inside a hopper that is an integral part of a vacuum chamber housing the roller and for example, E-beam (electron-beam) or a laser beam melting assembly. During operation the feedstock is poured over the rollers at a controlled rate using a regulator valve attached to the feeder. The vacuum chamber is desirably at a pressure ranging from 1 x 10⁻⁶ to 1 x 10⁻⁵ mBar during the operation.

The energy beam directed at the pellets heats and at least partially melts the titanium feedstock between the roller gap, which either softens it sufficiently for it to be deformed and consolidated as it passes through the roll gap, or melts it then solidifies it instantaneously on contacting the rollers and also gets deformed into a strip subsequently. The temperature of the solid strip coming out of the rollers is in the region of 600°C. Several titanium strips of dimensions in the range 300-900 mm (length) x 60-100 mm (width) x 3.0 mm (thickness) have been produced using this method.

This method is not specific only to titanium feedstock, it has potential application for direct production of strips of any metallic powder, and especially those that are very sensitive to the absorption of impurities such as oxygen or nitrogen.

The method of manufacture of strip described above is ideally suited to feed stock of uniformly sized granules of less than about 1 mm dimensions. Larger granules may be optimal for production of thicker sheets by this method.

Rollers are desirably cooled through the centre. The primary requirement is that the chamber housing the rollers should be in a vacuum (or very low pressure environment) to stop the molten titanium from picking up oxygen. A water-cooled roller assembly has been developed by the applicants that lets the water flow through the rollers and bearings, while maintaining good vacuum tightness.

For both variants of the invention described here for the production of metal alloy sheet and the production of shaped bar stock by energy beam heating of pellets or granular feed, the heating is conducted so as simultaneously to remove all or part of any volatile contamination that may be present in the feed material, for example, EDO granules may contain contaminants such as calcium chloride, calcium oxide or calcium metal.

## Claims

1. A method for purifying metal M₁ particles manufactured by an electrochemical reduction process, the method comprising the steps of:
introducing the metal M₁ particles into a heat source, such that the particles are out of contact with any surfaces, at a temperature substantially equal to or higher than the melting point of M₁ so as to cause vaporisation of some or substantially all of the contaminating impurities present;
removing the vaporised impurities from the vicinity of the particles;
and cooling the purified metal M₁ particles for collection in solid form.

2. A method for the manufacture of a metal alloy article containing a metal M₁, by purifying the metal M₁ particles using the method of Claim 1, and
performing a powder metallurgy process on the particles to form the article.

3. A method according to Claim 2 wherein the article is a metal alloy article, and in which the purified M₁ particles are mixed with particles of other alloy components and the powder metallurgy process is performed on the mixture to form the alloyed article.

4. A method as claimed in Claim 1, 2 or 3 wherein the particles are in the form of a powder.

5. A method according to Claim 4 wherein the powder comprises particles up to about 1 mm in diameter.

6. A method according to Claim 1, 2 or 3 wherein the particles are in the form of finely-sized metal samplers, granules or pellets.

7. A method according to any preceding claim wherein when the particles are out of contact with any surfaces, they are suspended in mid-air and/or permitted to free fall past or within the heat source.

8. A method according to any of Claims 1 to 6 wherein when the particles are out of contact with any surfaces they are entrained in a flame or blown through a plasma torch or are within an induction coil.

9. A method according to any preceding claim wherein the particles are heated, melted and substantially resolidified out of contact with any surfaces.

10. A method as claimed in any preceding claim wherein the free fall distance from the heat source is sufficiently long to allow any M₁ melted by the heat source to re-solidify before collection.

11. A method as claimed in any preceding claim wherein the heat source is selected from any one of a plasma torch, a laser, an electric arc, an induction coil or a tube furnace.

12. A method as claimed in any preceding claim, wherein the method is conducted in a controlled atmosphere.

13. A method as claimed in any preceding claim conducted in apparatus comprising a heat source, collection means for collecting the purified particles, and separate collection means for collecting the impurities.

14. A method as claimed in any preceding claim wherein the heat source is a plasma torch and the step of removing the vaporised impurities involves allowing the impurities to be swept away by the hot gas flow from the torch.

15. A method as claimed in any preceding claim wherein the temperature of the heat source is around or above the melting point, but below the boiling point of M₁.

16. A method according to any preceding claim wherein the metal M₁ particles for purification are manufactured by an electrochemical reduction process.

17. A method as claimed in any preceding claim wherein M₁ comprises titanium.

18. A method as claimed in any preceding claim wherein the impurities comprise one or more of magnesium, calcium and calcium chloride.

19. A method for the manufacture of a metal alloy article of uniform cross-section comprising the steps of:
introducing a continuous source of metal alloy M₁ pellets, containing contaminating impurities that are more volatile than M₁, to a processing means;
heating the pellets as they approach the processing means, by free-fall through a heat source, to a temperature substantially equal to or higher than the melting point of M₁ so as to cause vaporisation of some or substantially all of the contaminating impurities present;
removing the vaporised impurities from the vicinity of the pellets;
drawing the metal through the processing means so as to coalesce the pellets to form the desired article; and
cooling the cast stock.

20. A method as claimed in Claim 19 for the manufacture of a metal alloy sheet comprising the steps of:
introducing the continuous source of pellets to a pair of cooled feed rollers;
heating the pellets as specified in Claim 19 as they approach the nip of the pair of feed rollers;
drawing the metal through the nip of the rollers to form a sheet of metal alloy; and,
cooling the sheet.

21. A method as claimed in Claim 19 for the manufacture of a uniform cross-section metal alloy stock, comprising the steps of:
introducing the continuous source of pellets of the metal alloy to a shaped crucible;
heating the pellets as specified in Claim 19 as they approach the exposed surfaces of the crucible;
drawing the at least partially molten metal from an opposing surface of the crucible through a die, the die having a cross-section of near net shape and dimensions to the desired net shape and dimensions of the required stock; and,
cooling the cast stock.

22. A method as claimed in any of Claims 19 to 21, wherein the step of heating the pellets is carried out by means of an energy beam selected from an electron beam, a laser or a plasma torch.

23. A method as claimed in any of Claims 19 to 22, wherein the alloy substantially comprises titanium.

24. A method for fabricating purified metal particles comprising spherical particles with a reduced concentration of the volatile impurities using a method as defined in any of Claims 1 to 18.

25. A method according to Claim 24, wherein the concentration of the volatile impurities is less than 50ppm.

26. A method according to Claim 24 or 25, wherein the concentration of the volatile impurities is less than 10% of their concentration before purification.

## Patentansprüche

1. Verfahren zum Reinigen von Partikeln eines Metalls M₁, die mit einem elektrochemischen Reduktionsverfahren hergestellt wurden, wobei das Verfahren die folgenden Schritte beinhaltet:
Einleiten der Partikel des Metalls M₁ in eine Wärmequelle, so dass die Partikel mit keinen Flächen in Kontakt sind, bei einer Temperatur, die im Wesentlichen gleich oder höher als der Schmelzpunkt von M₁ ist, um zu bewirken, dass die vorhandenen kontaminierenden Verunreinigungen teilweise oder im Wesentlichen ganz verdampfen;
Beseitigen der verdampften Verunreinigungen aus der Nähe der Partikel;
und Kühlen der gereinigten Partikel des Metalls M₁, um sie in fester Form aufzufangen.

2. Verfahren zur Herstellung eines Metalllegierungsartikels, der ein Metall M₁ enthält, durch Reinigen der Partikel des Metalls M₁ mit dem Verfahren von Anspruch 1 und Ausführen eines Pulvermetallurgieverfahrens an den Partikeln zum Bilden des Artikels.

3. Verfahren nach Anspruch 2, wobei der Artikel ein Metalllegierungsartikel ist und wobei die gereinigten M₁-Partikel mit Partikeln anderer Legierungskomponenten gemischt werden und das Pulvermetallurgieverfahren an dem Gemisch zum Bilden des legierten Artikels ausgeführt wird.

4. Verfahren nach Anspruch 1, 2 oder 3, wobei die Partikel in Form eines Pulvers vorliegen.

5. Verfahren nach Anspruch 4, wobei das Pulver Partikel mit einem Durchmesser von bis zu etwa 1 mm umfasst.

6. Verfahren nach Anspruch 1, 2 oder 3, wobei die Partikel in Form von fein bemessenen Metallproben, Körnern oder Pellets vorliegen.

7. Verfahren nach einem der vorherigen Ansprüche, wobei die Partikel, wenn sie mit keinen Flächen in Kontakt sind, in der Luft suspendiert und/oder frei an der Wärmequelle vorbei oder darin fallen gelassen werden.

8. Verfahren nach einem der Ansprüche 1 bis 6, wobei die Partikel, wenn sie mit keinen Flächen in Kontakt sind, in einer Flamme mitgeführt oder durch einen Plasmabrenner geblasen werden oder sich innerhalb einer Induktionsspule befinden.

9. Verfahren nach einem der vorherigen Ansprüche, wobei die Partikel erhitzt, geschmolzen und im Wesentlichen ohne Kontakt mit Flächen wieder verfestigt werden.

10. Verfahren nach einem der vorherigen Ansprüche, wobei die Freifalldistanz von der Wärmequelle ausreicht, damit von der Wärmequelle geschmolzenes Metall M₁ vor dem Auffangen erneut verfestigen kann.

11. Verfahren nach einem der vorherigen Ansprüche, wobei die Wärmequelle ausgewählt wird aus der Gruppe bestehend aus einem Plasmabrenner, einem Laser, einem Lichtbogen, einer Induktionsspule oder einem Rohrofen.

12. Verfahren nach einem der vorherigen Ansprüche, wobei das Verfahren in einer geregelten Atmosphäre ausgeführt wird.

13. Verfahren nach einem der vorherigen Ansprüche, das in einer Vorrichtung ausgeführt wird, die eine Wärmequelle, ein Auffangmittel zum Auffangen der gereinigten Partikel und ein separates Auffangmittel zum Auffangen der Verunreinigungen beinhaltet.

14. Verfahren nach einem der vorherigen Ansprüche, wobei die Wärmequelle ein Plasmabrenner ist und der Schritt des Entfernens der verdampften Verunreinigungen das Wegreißenlassen der Verunreinigungen durch den Heißgasfluss von dem Brenner beinhaltet.

15. Verfahren nach einem der vorherigen Ansprüche, wobei die Temperatur der Wärmequelle um oder über dem Schmelzpunkt, aber unter dem Siedepunkt von M₁ liegt.

16. Verfahren nach einem der vorherigen Ansprüche, wobei die Partikel von Metall M₁ zur Reinigung durch ein elektrochemisches Reduktionsverfahren hergestellt werden.

17. Verfahren nach einem der vorherigen Ansprüche, wobei M₁ Titan umfasst.

18. Verfahren nach einem der vorherigen Ansprüche, wobei die Verunreinigungen Magnesium, Calcium und/oder Calciumchlorid beinhalten.

19. Verfahren zur Herstellung eines Metalllegierungsartikels mit gleichförmigem Querschnitt, das die folgenden Schritte beinhaltet:
Zuführen eines kontinuierlichen Vorrats von Pellets aus einer Metalllegierung M₁, die kontaminierende Verunreinigungen enthalten, die flüchtiger sind als M₁, zu einem Verarbeitungsmittel;
Erhitzen der Pellets bei ihrer Annäherung an das Verarbeitungsmittel durch freien Fall durch eine Wärmequelle bis auf eine Temperatur, die im Wesentlichen gleich oder höher als der Schmelzpunkt von M₁ ist, um eine Verdampfung von einigen oder im Wesentlichen allen der vorhandenen kontaminierenden Verunreinigungen zu bewirken;
Entfernen der verdampften Verunreinigungen aus der Nähe der Pellets;
Ziehen des Metalls durch das Verarbeitungsmittel, um die Pellets zu dem gewünschten Artikel zu koaleszieren; und
Kühlen des gegossenen Produkts.

20. Verfahren nach Anspruch 19 zur Herstellung eines Metalllegierungsblechs, das die folgenden Schritte beinhaltet:
Zuführen des kontinuierlichen Pelletvorrats zu einem Paar gekühlten Zuführungswalzen;
Erhitzen der Pellets gemäß Anspruch 19 bei ihrer Annäherung an den Walzenspalt des Zuführungswalzenpaares;
Ziehen des Metalls durch den Spalt der Walzen, um ein Metalllegierungsblech zu bilden; und
Kühlen des Blechs.

21. Verfahren nach Anspruch 19 zur Herstellung eines Metalllegierungsmaterials mit gleichförmigem Querschnitt, das die folgenden Schritte beinhaltet:
Zuführen des kontinuierlichen Pelletvorrats aus der Metalllegierung zu einem gestalteten Schmelztiegel;
Erhitzen der Pellets nach Anspruch 19 bei ihrer Annäherung an die exponierte Oberfläche des Schmelztiegels;
Ziehen des wenigstens teilweise geschmolzenen Metalls von einer gegenüberliegenden Fläche des Schmelztiegels durch eine Düse, wobei die Nettoform und die Nettoabmessungen des Querschnitts der Düse nahezu der/den gewünschten Nettoform und -abmessungen des gewünschten Materials entsprechen; und
Kühlen des Gussteils.

22. Verfahren nach einem der Ansprüche 19 bis 21, wobei der Schritt des Erhitzens der Pellets mit einem Energiestrahl ausgeführt wird, der aus einem Elektronenstrahl, einem Laser oder einem Plasmabrenner ausgewählt wird.

23. Verfahren nach einem der Ansprüche 19 bis 21, wobei die Legierung im Wesentlichen Titan umfasst.

24. Verfahren zur Herstellung von gereinigten Metallpartikeln, die sphärische Partikel mit einer reduzierten Konzentration der flüchtigen Verunreinigungen unter Anwendung eines Verfahrens nach einem der Ansprüche 1 bis 18 beinhaltet.

25. Verfahren nach Anspruch 24, wobei die Konzentration der flüchtigen Verunreinigungen weniger als 50 ppm beträgt.

26. Verfahren nach Anspruch 24 oder 25, wobei die Konzentration der flüchtigen Verunreinigungen weniger als 10% der Konzentration vor dem Reinigen ausmacht.

## Revendications

1. Procédé de purification de particules de métal M₁ fabriquées par un processus de réduction électrochimique, le procédé comprenant les étapes suivantes:
introduction des particules de métal M₁ dans une source de chaleur, de telle sorte que les particules ne soient en contact avec aucune surface, à une température sensiblement égale ou supérieure au point de fusion de M₁ de façon à provoquer la vaporisation de certaines ou sensiblement de toutes les impuretés contaminantes présentes;
élimination des impuretés vaporisées du voisinage des particules;
et refroidissement des particules de métal M₁ purifiées pour leur collecte sous forme solide.

2. Procédé de fabrication d'un article en alliage métallique contenant un métal M₁, en purifiant les particules de métal M₁ au moyen du procédé de la revendication 1, et
en exécutant un processus de métallurgie des poudres sur les particules afin de former l'article.

3. Procédé selon la revendication 2, dans lequel l'article est un article en alliage métallique, et dans lequel les particules M₁ purifiées sont mélangées à des particules d'autres composants d'alliage et le processus de métallurgie des poudres est exécuté sur le mélange afin de former l'article allié.

4. Procédé selon la revendication 1, 2 ou 3, dans lequel les particules se présentent sous forme de poudre.

5. Procédé selon la revendication 4, dans lequel la poudre comprend des particules mesurant jusqu'à 1 mm de diamètre.

6. Procédé selon la revendication 1, 2 ou 3, dans lequel les particules se présentent sous forme d'échantillons, de granulés ou de boulettes métalliques très fins.

7. Procédé selon l'une quelconque des revendications précédentes, dans lequel quand les particules ne sont en contact avec aucune surface, elles sont en suspension dans l'air et/ou peuvent tomber en chute libre devant ou dans la source de chaleur.

8. Procédé selon l'une quelconque des revendications 1 à 6, dans lequel quand les particules ne sont en contact avec aucune surface, elles sont entraînées dans une flamme ou soufflées à travers un chalumeau à plasma ou se trouvent dans une bobine d'induction.

9. Procédé selon l'une quelconque des revendications précédentes, dans lequel les particules sont chauffées, fondues et sensiblement resolidifiées pour ne faire contact avec aucune surface.

10. Procédé selon l'une quelconque des revendications précédentes, dans lequel la distance de chute libre depuis la source de chaleur est suffisamment longue pour permettre à tout M₁ fondu par la source de chaleur de se resolidifier avant la collecte.

11. Procédé selon l'une quelconque des revendications précédentes, dans lequel la source de chaleur est sélectionnée indifféremment parmi un chalumeau à plasma, un laser, un arc électrique, une bobine d'induction et un four à tube.

12. Procédé selon l'une quelconque des revendications précédentes, dans lequel le procédé est effectué dans une atmosphère contrôlée.

13. Procédé selon l'une quelconque des revendications précédentes effectué dans un appareil comprenant une source de chaleur, un moyen de collecte pour collecter les particules purifiées, et un moyen de collecte séparé pour collecter les impuretés.

14. Procédé selon l'une quelconque des revendications précédentes, dans lequel la source de chaleur est un chalumeau à plasma et l'étape de retrait des impuretés implique l'élimination des impuretés par balayage par le flux de gaz chaud provenant du chalumeau.

15. Procédé selon l'une quelconque des revendications précédentes, dans lequel la température de la source de chaleur se situe autour ou au-dessus du point de fusion, mais en dessous du point d'ébullition de M₁.

16. Procédé selon l'une quelconque des revendications précédentes, dans lequel les particules de métal M₁ à purifier sont fabriquées par un processus de réduction électrochimique.

17. Procédé selon l'une quelconque des revendications précédentes, dans lequel M₁ comprend le titane.

18. Procédé selon l'une quelconque des revendications précédentes, dans lequel les impuretés comprennent un ou plusieurs du magnésium, du calcium et du chlorure de calcium.

19. Procédé de fabrication d'un article en alliage métallique d'une coupe transversale uniforme, comprenant les étapes suivantes:
introduction d'une source continue de boulettes d'alliage métallique M₁, contenant des impuretés contaminantes qui sont plus volatiles que M₁, dans un moyen de traitement;
chauffage des boulettes lorsqu'elles approchent du moyen de traitement, par chute libre à travers une source de chaleur, à une température sensiblement égale ou supérieure au point de fusion de M₁ de façon à provoquer la vaporisation de certaines ou sensiblement de toutes les impuretés contaminantes présentes;
élimination des impuretés vaporisées du voisinage des boulettes;
étirage du métal à travers le moyen de traitement de façon à coalescer les boulettes afin de former l'article souhaité; et
refroidissement de la masse coulée.

20. Procédé selon la revendication 19 de fabrication d'une tôle en alliage métallique comprenant les étapes suivantes:
introduction de la source continue de boulettes dans une paire de rouleaux d'alimentation refroidis;
chauffage des boulettes comme cela est spécifié à la revendication 19 quand elles approchent de la zone de pincement de la paire de rouleaux d'alimentation;
étirage du métal à travers la zone de pincement des rouleaux afin de former une tôle d'alliage métallique; et,
refroidissement de la tôle.

21. Procédé selon la revendication 19 de fabrication d'une masse d'alliage métallique de coupe transversale uniforme comprenant les étapes suivantes:
introduction de la source continue de boulettes de l'alliage métallique dans un creuset conformé;
chauffage des boulettes comme cela est spécifié à la revendication 19 quand elles approchent de la surface exposée du creuset;
étirage du métal au moins partiellement fondu depuis une surface opposée du creuset à travers une filière, la filière ayant une coupe transversale d'une forme presque nette et des dimensions correspondant à la forme nette souhaitée et aux dimensions de la masse requise; et
refroidissement de la masse coulée.

22. Procédé selon l'une quelconque des revendications 19 à 21, dans lequel l'étape de chauffage des boulettes est exécutée au moyen d'un faisceau d'énergie sélectionné parmi un faisceau d'électrons, un laser ou un chalumeau à plasma.

23. Procédé selon l'une quelconque des revendications 19 à 22, dans lequel l'alliage comprend essentiellement du titane.

24. Procédé de fabrication de particules métalliques purifiées comprenant des particules sphériques à concentration réduite d'impuretés volatiles au moyen d'un procédé tel que défini dans l'une quelconque des revendications 1 à 18.

25. Procédé selon la revendication 24, dans lequel la concentration d'impuretés volatiles est inférieure à 50 ppm.

26. Procédé selon la revendication 24 ou 25, dans lequel la concentration d'impuretés volatiles est inférieure à 10% de leur concentration avant purification.
